

(No Model.)

H. L. HAAS.  
PROCESS OF NICKEL PLATING.

No. 564,748.

Patented July 28, 1896.



WITNESSES:

John Bergendy  
James Cosgrave

INVENTOR,

Harry L. Haas,  
BY  
Botts, Hyde & Botts

ATTORNEYS

# UNITED STATES PATENT OFFICE.

HARRY L. HAAS, OF NEW YORK, N. Y., ASSIGNOR TO THE ZUCKER & LEVETT & LOEB COMPANY, OF SAME PLACE.

## PROCESS OF NICKEL-PLATING.

SPECIFICATION forming part of Letters Patent No. 564,748, dated July 28, 1896.

Application filed November 27, 1895. Serial No. 570,291. (No specimens.)

*To all whom it may concern:*

Be it known that I, HARRY L. HAAS, of the city, county, and State of New York, have invented certain new and useful Improvements 5 in Processes of Nickel-Plating, of which the following is a specification, reference being had to the accompanying drawing.

My invention relates to improvements in the art of nickel-plating, the objects being, 10 first, to more quickly accomplish the plating than heretofore; second, to use an electric current of small voltage; third, to more uniformly, as regards thickness, adhesion, and color, accomplish the depositing of nickel 15 upon the cathode, and, fourth, to render unnecessary the addition, during the plating operation, of nickel-salts to strengthen the plating-bath, as heretofore.

In the accompanying drawing there is 20 shown a partly-sectional view of a nickel-plating bath, the source of electrical energy, which may be of any useful form, being omitted.

In the accompanying drawing I have shown 25 one form of apparatus which may be employed in carrying out my new process of nickel-plating.

A represents the box for containing the electrolyte or solution B. A suspended anode C, of nickel, is partly immersed in the solution. 30 This anode differs from those used prior to my invention, in that it presents to the electrolyte a much greater surface than is presented by a plane flat anode of the same length and breadth, and although other forms of nickel 35 anodes constructed so as to have an increased surface may be employed with advantage, yet I prefer to use a corrugated anode made substantially as shown in the accompanying drawing. This anode is suspended from a 40 metallic rod D by means of hooks F F, and is connected by conductor E to the positive pole of the generator. The metallic rod G, from which the cathode is suspended, is connected to the negative pole of such generator.

45 During electrolysis both the sulfate of nickel and the sulfate of ammonia are decomposed, and sulfuric acid and ammonia are set free at the anode. The sulfuric acid forms an equivalent quantity of sulfate of nickel by 50 its action on the anode, which it dissolves.

If the amount of ammonia freed at the

anode becomes too great, in proportion to the amount of sulfuric acid set free, the solution will, in a short time, become weak in metal and decidedly alkaline, and it has been found 55 that the more intense the current of electricity employed the more rapid will be the uneven liberation of the ammonia and sulfuric acid, which will cause the quality of the deposit of the nickel upon the cathode to be- 60 come gradually poorer in color and inadhesiveness, because it has been found that the more intense the electric current the more hydrogen is eliminated, which makes the deposit upon the cathode brittle and strip, especially 65 if the deposit is thick.

By the employment of an anode of nickel, which presents to the electrolyte a much greater surface than would be the case if a plane anode were used, I find that an elec- 70 tric current of very low intensity may be employed, even as low as two volts, and that such current may be more uniformly maintained and that less ammonia is liberated than when the plane anode is used, and I 75 find also that a much greater amount of nickel is dissolved from the corrugated anode because of the increased surface presented, and that the strength of the bath is more uniformly maintained, with the direct result that 80 the nickel deposited upon the cathode is more regular and uniform in color and thickness, adheres more tenaciously, and does not scale therefrom, as was the case heretofore, due to excess of hydrogen at the cathode by the de- 85 posited nickel. Furthermore, I have found that with the use of a corrugated anode the action of the gases formed at the anode is quite different from that which occurs when a plane or flat anode is used. With a plane 90 or flat anode the gases developed at the anode are apt to proceed in considerable quantities directly across to the cathode, and their presence at the cathode acts deleteriously upon the deposit of nickel, as the nickel is apt to 95 be flaky and non-adherent. On the other hand, with a corrugated anode, the gases are developed on surfaces which are inclined to each other, and the gas developed on one surface meets that developed on the surface in- 100 clined to it, and instead of proceeding in any marked quantity across to the cathode it

forms into bubbles, which rise to the surface of the solution. As a result of this action the deposit of nickel is whiter and more malleable when a corrugated anode is used than when a plane or flat anode is used, the other conditions being the same.

I have also discovered that, when the anode presenting an increased surface is not used, the strength of the solution will not be uniform, for, if the anode-surface is not considerably larger than that of the article to be deposited upon, more nickel will be deposited on the work than is dissolved from the anode, and all the sulfuric acid which is evolved at the anode will not be dissolved to form sulfate of nickel, but will combine with some of the ammonia, and the bath will become, in time, composed of sulfate of ammonia and very little sulfate of nickel, thereby weakening the solution in nickel and causing the deposit to become dark in color. To overcome this objection, it was customary to add nickel-salts to the solution, as required, but, by the use of my process, the addition of such salts is rendered unnecessary, due to the evenness existing between the resolving of the anode into the solution and the deposition of nickel upon the cathode. I have also found that when an anode having the increased surface is employed the increased size of the anode and its more even solution into the bath contribute to make the electrolyte a much better conductor of the current than when the plane anode is employed, the objection heretofore being that as the solution becomes weaker in nickel the resistance to the passage of the current was increased, and this difficulty rendered necessary the employment of a current much higher in voltage than is required in connection with any new process of plating, which has been objectionable and expensive.

One of the disadvantages due to the employment of currents of high voltage is the tendency of the nickel to precipitate in the form of basic salt, impairing the metallic strength of the bath. This precipitation I prevent by the employment of a current of low voltage and an anode presenting a greatly increased surface to the solution. The process of nickel-plating therefore differs from most, if not all, other plating processes in that a substantially neutral solution must be employed, which renders the rate of solution of the anode comparatively slow and unequal to the rate of deposit at the cathode, and this results in the necessity of constantly replenishing the solution with salts of nickel to maintain the requisite strength of the solution. These difficulties are remedied by my invention and the process rendered substantially even and continuous as long as the anode lasts.

I am aware of the United States Letters Patent to W. H. Remington, dated October 6, 1868, No. 82,877, and to A. C. Wenzel, dated September 10, 1878, No. 208,003, both of which

show and describe anodes composed of boxes having perforated sides and bottoms and containing nickel in the form of grains, and I especially disclaim the forms of anodes shown and described in the said patents as being entirely unfitted for the purposes of my invention, because of the imperfect electrical and mechanical contact between the grains, which results in the formation of an anode offering an enormous resistance to the passage of electricity. My invention, on the contrary, contemplates the employment of a continuous solid anode.

I am also aware of the United States Letters Patent to D'Humy, No. 367,705, dated August 2, 1887, for galvanic battery, which shows a corrugated element of iron or steel, and I especially disclaim from my invention the use of elements of iron or steel, and in fact all metals excepting those which are wholly or largely composed of nickel or an alloy thereof. I desire also to call attention to the fact that the D'Humy patent does not describe any process of plating, and the uses and construction of my invention are quite different.

I am also aware of United States Letters Patent No. 317,246, dated May 5, 1885, to E. P. Thompson, for an apparatus for the electrodeposition of gold from its chlorids, and I disclaim the apparatus and process there described, which cannot be used for the same purposes as my invention and which are different in material and important respects therefrom.

I also desire to be understood as not attempting to cover the use of plane flat anodes of nickel, which cannot advantageously be employed, requiring an unnecessary and undesirable enlargement of the size of the bath or a reduction of the quantity of the electrolyte.

I am also aware of what is disclosed in British Patent No. 3,533, of February 27, 1889, for improvements in the extraction of copper, zinc, and precious metals by electrolysis, in which, among other things, it is proposed to use an anode which may consist of pieces or plates of retort-carbon, conveniently shaped and in electric connection with each other, or perforated lead plates covered with small pieces of retort-carbon, or of lead plates with rather deep corrugations, likewise perforated to allow the liquid to pass through the plates, and make no claim thereto, as these would not be practicable for the purposes of my invention, nor would they, or any of them, accomplish the results stated above.

Having described my invention, what I claim, and desire to secure, is—

The process of nickel-plating herein described, which consists in employing, in a substantially neutral solution, a continuous solid anode having a corrugated or equivalently-extended surface, which is greater than would be presented by an anode of the same length and breadth but having a plane sur-

face, and then passing an electric current through the anode and the solution, and, by the use of such anode, balancing the solution of the anode and the deposit at the cathode, whereby the metallic strength of the solution is maintained substantially uniform, substantially as and for the purpose described.

In witness whereof I have heretunto subscribed my name this 25th day of November, 1895.

HARRY L. HAAS.

In presence of—

Wm. H. BERRIGAN, Jr.,  
W. S. JONES.